

## 1

3,394,082

### CUBIC FERRITE WITH A HIGH UPPER FREQUENCY LIMIT

Mieczyslaw Hildebrandt, Jean Nicolas, and Avénir Vassiliev, Paris, France, assignors to CSF—Compagnie Générale de Télégraphie Sans Fil, a corporation of France

No Drawing. Filed Oct. 27, 1964, Ser. No. 406,887  
Claims priority, application France, Oct. 30, 1963,

952,267

1 Claim. (Cl. 252—62.58)

#### ABSTRACT OF THE DISCLOSURE

The invention concerns cubic lithium ferrites used in application involving scalar permeability and defined by the formula

$\frac{1}{4}\{\text{Li}_2\text{O}; 4.5[(1-x)\text{Fe}_2\text{O}_3, x\text{Al}_2\text{O}_3]\}; 2y\text{MnO}_2; z\text{CoO}$

wherein:

$x$  lies between 0 and 0.25

$y$  lies between 0.15 and 0.6

$z$  lies between 0.04 and 0.35

The ferrites according to the invention have a higher frequency limit than conventional ferrites.

The present invention, relates to cubic lithium ferrites.

These materials are used in applications involving scalar permeability, for example for the fabrication of magnetic cores.

Known materials of this kind have an upper frequency  $f_L$  of the order of a few tens of mc./s., at which relaxation phenomena cause a rapid rise of magnetic loss and lowering of the initial permeability.

It is an object of this invention to provide ferrites with a higher frequency limit than conventional ferrites. The ferrites according to the invention have a composition defined by the formula:

$\frac{1}{4}\{\text{Li}_2\text{O}; 4.5[(1-x)\text{Fe}_2\text{O}_3, x\text{Al}_2\text{O}_3]\}; 2y\text{MnO}_2; z\text{CoO}$

wherein:

$x$  lies between 0 and 0.25

$y$  lies between 0.15 and 0.6

$z$  lies between 0.04 and 0.35.

The invention will be better understood from the following description of the method of manufacture of a ferrite.

The raw materials used are the compounds  $\text{Fe}_2\text{O}_3$ ,  $\text{Al}_2\text{O}_3$ ,  $\text{MnO}_2$ ,  $\text{CO}_3\text{Li}_2$  and  $\text{CoO}$  with a degree of purity higher than 99.5%. The compounds are proportioned by weight, crushed in distilled water for 24 hours in steel ball-mills and dried. The resulting mixture is pre-sintered at 800° C. for 2 hours and crushed once more as above. When dried, the powder is transformed to a granulate by adding 15% by weight of aqueous polyvinyl alcohol solution. The granulate is pressed at a pressure of 1 ton

## 2

per  $\text{cm}^2$ . The resulting parts are sintered for 3 hours at a temperature  $T_f$  between 1100° and 1200° C.

Of course, certain details of the process can be varied without departing from the spirit of the invention. However, it is to be noted that the sintering temperature is relatively critical.

If the sintering temperature is less than 1100° C., the resulting material is crumbly. If the temperature is above 1200° C., the material decomposes.

The following table shows the characteristics of the material obtained, against parameters  $x$ ,  $y$  and  $z$  and temperature  $T_f$ ,  $\mu$  being the initial permeability:

| Example No. | $x$  | $y$  | $z$    | $T_f$ | $\mu$ | $f_L$ mc./s. |
|-------------|------|------|--------|-------|-------|--------------|
| 1           | 0    | 0.61 | 0.201  | 1,100 | 7     | 100          |
| 2           | 0    | 0.6  | 0.268  | 1,100 | 5     | 150          |
| 3           | 0    | 0.6  | 0.335  | 1,100 | 4     | 200          |
| 4           | 0.05 | 0.6  | 0.201  | 1,100 | 7     | 110          |
| 5           | 0.05 | 0.6  | 0.268  | 1,100 | 4.8   | 160          |
| 6           | 0.05 | 0.6  | 0.335  | 1,100 | 4.6   | 190          |
| 7           | 0.1  | 0.6  | 0.134  | 1,100 | 8     | 110          |
| 8           | 0.1  | 0.6  | 0.201  | 1,100 | 6.5   | 190          |
| 9           | 0.1  | 0.6  | 0.268  | 1,100 | 5     | 150          |
| 10          | 0.1  | 0.6  | 0.335  | 1,100 | 4     | 160          |
| 11          | 0.15 | 0.6  | 0.0402 | 1,100 | 7     | 100          |
| 12          | 0.15 | 0.6  | 0.201  | 1,100 | 5     | 150          |
| 13          | 0.15 | 0.6  | 0.268  | 1,100 | 4     | 150          |
| 14          | 0.15 | 0.6  | 0.335  | 1,100 | 3.8   | 200          |
| 15          | 0    | 0.6  | 0.201  | 1,150 | 8     | 100          |
| 16          | 0    | 0.6  | 0.268  | 1,150 | 5.6   | 150          |
| 17          | 0    | 0.6  | 0.335  | 1,150 | 5.6   | 150          |
| 18          | 0.05 | 0.6  | 0.268  | 1,150 | 5.4   | 150          |
| 19          | 0.05 | 0.6  | 0.335  | 1,150 | 4.2   | 200          |

What is claimed is:

1. A ferrite composition having low losses in the frequency range between 50 and 200 mc./s. defined by the formula:

$\frac{1}{4}\{\text{Li}_2\text{O}; 4.5[(1-x)\text{Fe}_2\text{O}_3, x\text{Al}_2\text{O}_3]\}; 2y\text{MnO}_2; z\text{CoO}$

wherein:

$0 \leq x \leq 0.25$

$0.15 \leq y \leq 0.6$

$0.04 \leq z \leq 0.35$

#### References Cited

##### UNITED STATES PATENTS

|           |         |                        |          |
|-----------|---------|------------------------|----------|
| 2,958,664 | 11/1960 | Vassiliev et al. ----- | 252—62.5 |
| 3,007,874 | 11/1961 | Peyssou et al. -----   | 252—62.5 |
| 3,030,307 | 4/1962  | Baird et al. -----     | 252—62.5 |
| 3,066,103 | 11/1962 | Owen -----             | 252—62.5 |
| 3,072,576 | 1/1963  | Greenhouse -----       | 252—62.5 |
| 3,232,877 | 2/1966  | Vassiliev et al. ----- | 252—62.5 |
| 3,245,911 | 4/1966  | Vassiliev et al. ----- | 252—62.5 |

#### OTHER REFERENCES

Aghajanian: "High Curie Temperature Square Loop Ferrites," IBM Technical Disclosure Bulletin, page 85, volume 4, No. 12, May 1962.

TOBIAS E. LEVOW, Primary Examiner.

R. D. EDMONDS, Assistant Examiner.